

1

3,350,218

## SOILPROOFING WITH QUATERNARY AMMONIUM DERIVATIVES OF HIGHLY FLUORINATED CARBOXYLIC ACIDS

Domenick Donald Gagliardi, East Greenwich, R.I., assignor to Colgate-Palmolive Company, New York, N.Y., a corporation of Delaware

No Drawing. Filed Sept. 13, 1963, Ser. No. 308,631  
10 Claims. (Cl. 117—76)

The present invention relates to "soilproofing" textiles and to the "soilproofing" quaternary ammonium compounds used and more particularly, to "soilproofing" textiles with quaternary ammonium compounds from highly fluorinated carboxylic acids and to the quaternary ammonium compounds from highly fluorinated carboxylic acids per se.

For centuries man has sought to alleviate the discomfort concomitant with exposure to rain. One hundred years ago MacIntosh provided the coated fabric which has, in subsequent years, provided a generic name for a particular class of rainwear. It was not until about 1935 that there was any attempt to discover the factors controlling resistance to wetting by water. Prior to this time, textile materials were coated fabrics with various "cookbook" recipes such as rubber, linseed oil-rubber mixtures, empirical and whimsical synthetic dopes and other compositions having no basis in a discovery of the physical properties of a preparation which would impart to a textile the capability of water repellency. Without understanding the basic principles of surface free energy, contact angle, and spreading coefficient several unrelated practical developments arose during the half-decade from 1935 to 1940 which changed the art of water-proofing textiles. In Germany, a series of paraffin wax emulsions were developed which, when padded onto textiles, produced a high contact angle of water drops on the surface and a high degree of shower resistance without changing the porosity or air permeability of the textile material as do the preparations recommended for waterproofing prior to 1935. The treated fabrics were non-wettable by water and water-borne liquids and stains because of the change of the free energy of the fiber surfaces and not because the interstices of the woven fabrics were plugged. Thus, a practical improvement was made without an understanding of the reason for the advance in the art.

By the use of these new wax emulsion-metallic salts mixtures, it was then and is now possible to produce fabrics which have the feel and appearance of conventional fabrics but do not look like oil-cloths or fabrics having rubberized coating. The only practical limitation of such mixtures is the durability to washing and drycleaning. This class of water-proofing materials generally comprise a mixture containing:

(a) A paraffin wax or mixtures of vegetable wax esters such as carnauba, candelilla, or sugar cane wax.

(b) An emulsifying agent, usually glue, gelatin, and rosin soaps.

(c) An aluminum or zirconium salt, usually the formate or acetate. The primary function of the salt is to insolubilize the glue and other emulsifiers after the emulsion is deposited on the fabric.

A large variety of such products are still in use as low-cost, non-durable water repellents for textiles. Since neither thermosetting nor fiber reaction occurs when textiles are coated with such products, the treated textile is non-durable to washing and dry cleaning. Other than water repellency for rainwater fabrics, such mixtures provide fabrics with a fair degree of spot and stain resistance to water-borne chromophoric materials.

2

The search for durable or permanent water repellents as contrasted with these non-durable water repellents, especially for cellulosic fibers was initiated by the need to overcome the deficiencies of these wax emulsion-metallic salt mixtures. The first major advance occurred in England where a product marketed under the trade name "Velan" was produced. This material was octadecyloxy-methyl pyridinium chloride, a quaternary ammonium compound made by the chloromethylation of octadecanol, followed by quaternization with pyridine to yield a product having a composition represented by the formula



This compound, unlike other quaternaries, is unstable and under acid conditions reacts with surfaces containing active hydrogen, e.g., the hydrogen of a hydroxyl group in cellulose fibers. If the cellulose molecules be represented by  $\text{Z}(\text{OH})_n$  then the reaction can be considered to be summarized by the equation:



where  $\text{py}$  is the balance of the pyridine ring. Fabrics treated with such a compound are durably water repellent, are porous, soft, and have the appearance of untreated fabrics.

A major improvement of the "Velan" type material was made when the stearamidomethyl analog of "Velan"



commercially known as "Zelan" and "Norane R" was produced. The advantage of the stearamide product is greater initial water repellency and greater durability to washing. Such products are still among the forefront of the leaders in rainwear fabric finishes.

In the search for other fabric-reactive or durable water repellents other classes of compounds have been developed. Illustrative of these other classes of water repellents are the silicone water repellents methylstearamide compositions ("Permel," "Ahcovel NW"), hydrophobic resins ("Norane GG," "Ranedare R," "Argus DWR"), octadecylgutene dimer ("Aquapel") and others.

While durable water repellents had been initially developed for outerwear and raincoat applications, it was soon recognized that durable water repellents could be used as finishes for other purposes. In the period 1950 to 1956 these durable water repellent finishes were widely used on men's suitings, dress goods, and upholstery materials. When offering these products to the textile finishing trade, promotional emphasis was not placed on water-repellency but on spot-and-stain resistance. This use has continued to the present time. It had been observed that fabrics treated with such durable water repellents had a high degree of resistance to soiling by water-borne soils and stains and were easier to launder. The primary limitation of these finishes was that they attracted rather than repelled oily soils, and the treated fabrics were not resistant to staining by oily materials such as oils, greases, gravy, mayonnaise, etc.

In the early part of the 1950 decade based on work done at Naval Research Laboratory by Fox and Zisman and from work done at a division of the Minnesota Mining and Manufacturing Co., the utility of certain fluorocarbon based chemicals as fibrous finishes was announced. Fox and Zisman had demonstrated the physicochemical principle of low free energy surfaces and the

relation of non-wetting with water or oils of surfaces treated with chemicals containing perfluoroalkyl groups.

The practical developments of "3M" culminated in the introduction of the first product for textile treating. This product is still known as FC-149 and is a classical Werner complex of a carboxylic acid made by reacting one mol of the acid with two mols of basic chromic chloride. The compound is water soluble and cationic in nature. It exhibits strong adhesion to anionic substrates such as cellulose and fiberglass. It also complexes with proteinaceous fibers such as wool, silk, and leather to give both water and oil repellent surfaces. It is generally believed that perfluorodecanoic acid is the base for this product.

Subsequently, "3M" made a product known as FC-208 available as a finish. It is generally believed that this finishing material is a perfluorosulfonamide having a composition corresponding to the formula



where  $x$  is an integer in the range of 3 to 13,  $\text{R}'$  is methyl, ethyl, propyl, butyl, amyl, hexyl,  $\text{R}''$  is an alkylene radical having 1 to 12 carbon atoms and  $\text{R}'''$  is hydrogen, methyl, or ethyl.

The advent of these "perfluoro" finishes produced a great practical improvement in fabric finishes. Although of little merit for plain water repellency for outerwear purposes, the two products, i.e., the Werner Complex and the perfluorosulfonamide, offer a solution to the problem of providing fabrics with water-and-oil repellency and practical resistance to staining. Because of its hydrolytic instability the Werner complex has been limited to wool, leather, and upholstery finishes. The sulfonamide has become a leader in finishes for cotton, rayon, and non-cellulosic synthetic fiber.

Important as water-and-oil repellency and resistance to staining by water-and-oil borne stains are for wearing apparel, upholstery and the like, the capability of shedding oily particulate soil is of greater importance. That is to say, the finely divided environmental grime mixed with the oil exudations of the human skin, i.e., oily particulate soil, which soil the neckband and cuffs of a man's shirt are far more often encountered than soiling with gravy or mayonnaise. Hence, while fabric finishes which repel water, oil, water-borne and oil-borne stains are of great importance, the capability of resisting staining by oily particulate soil is of greater importance for aesthetic reasons if for no other reason. Yet even the "perfluoro" finishes presently available do not have the capability of resisting staining by oily particulate soil. In fact, they enhance such soiling.

It is manifest that controlled evaluating of fabric finishes in actual use is not possible. Consequently, it has been necessary to use evaluation methods subject to laboratory control which will simulate as closely as possible actual conditions under which water-repellency, oil-repellency, resistance to staining by water-borne and oil-borne stains, and resistance to staining by oily particulate soil of treated fabrics occurs. Such methods of evaluation are the following.

*Water Repellency (resistance to wetting (spray test)  
AATCC Standard Test Method 22-1952)*

This test is applicable to any textile fabric. It measures the resistance of fabrics to wetting by a water spray and the results depend primarily on the degree of hydrophobicity inherent in the fibers and yarns and subsequent treatments to which the fabric is subjected. Water is sprayed against the taut surface of a test specimen. Evaluation of the wetted pattern is readily brought about by comparing the wetted pattern with standard wetting pattern pictures:

|    | Characterized by:                                                 | Rating |
|----|-------------------------------------------------------------------|--------|
|    | No sticking or wetting of the upper surface                       | 100    |
| 5  | Slight random sticking or wetting of the upper surface            | 90     |
|    | Wetting of the upper surface at spray points                      | 80     |
| 10 | Partial wetting of the whole of the upper surface                 | 70     |
|    | Complete wetting of the whole of the upper surface                | 50     |
| 15 | Complete wetting of the whole of the upper and the lower surfaces | 0      |

The test specimens of minimum size of 7" x 7" (seven inches by seven inches) are conditioned at 70° F. and 65 percent relative humidity for a minimum of four hours before testing.

The test specimen, fastened securely and wrinkle-free in a metal hoop having a diameter of 6 inches, is placed and centered 6 inches under a standard spray nozzle at an angle of 45° to the horizontal. Two hundred and fifty 20 milliliters of water at 80±2° F. is poured into a funnel attached above the spray nozzle. The spray lasts 25 to 30 seconds at the end of which time the hoop is taken by one edge and the opposite edge tapped smartly once against a solid object with the wet side facing the solid; this procedure is repeated with the hoop reversed 180°.

*Oil Repellency ("3M Textile Chemicals" Appendix A—Test Methods, page 1)*

The Minnesota Mining oil repellency test is based on 30 the different penetrating properties of the two hydrocarbon liquids, mineral oil ("Nujol") and n-heptane. ("Nujol" is the trade name for white mineral or paraffin oil being a mixture of hydrocarbons having a density for "light" oil in the range of 0.83 to 0.860 and for "heavy" 35 oil in the range of 0.875 to 0.905.) The "Nujol"-heptane proportions for each rating were selected by "3M" to give oily stain resistance somewhat comparable to the water-borne strain resistance corresponding to each of the spray ratings of the AATCC Standard Test Method 22-1952.

| Oil Repellency Rating | Percent Heptane (by volume) | Percent "Nujol" (by volume) |
|-----------------------|-----------------------------|-----------------------------|
| 100+                  | 60                          | 40                          |
| 100                   | 50                          | 50                          |
| 90                    | 40                          | 50                          |
| 80                    | 30                          | 70                          |
| 70                    | 20                          | 80                          |
| 50                    | 0                           | 100                         |
| 0                     | -----                       | ( <sup>1</sup> )            |

<sup>1</sup> No hold out to "Nujol".

The standard oil-heptane mixtures are contained in 55 small stoppered medicine-dropper bottles. A drop of each mixture of "Nujol" and heptane is placed on the fabric. The appearance of the test oil is observed through the drop. Note is made whether wetting or penetration occurs. The number corresponding to that mixture containing the highest percentage of heptane which does not penetrate or wet the fabric after three minutes is considered the oil repellency rating of the system.

60 The change in the optical refractivity of the drop is often an indication of wetting. In some cases wetting can be better determined by observing the other side of the fabric. In some cases reported hereinafter the term "0+" has been used to indicate a modicum of resistance to 65 wetting by oil.

*Stain repellency*

The following procedures have been used to establish 70 the degree of resistance to starting by water-borne and oil-borne stains of fabrics.

(a) The fabrics were stretched lightly on 12" x 31" frames. All or part of the frame was used depending upon the amount of fabric available. The frames were supported at both ends with the fabric about 8 inches above 75 a black surface. The fabric touched nothing.

(b) Three inch medicine droppers were used to draw the stains from the containers. A 1 cubic centimeter calibration was established and marked on the exterior of each dropper. The stains were squeezed vertically downward from a height 2 inches above the cloth.

(c) After five minutes the unabsorbed stain was wiped off the fabric with two sweeps of "Kleenex" and the stains rated as follows.

| Appearance:             | Rating |
|-------------------------|--------|
| No stain visible        | 5      |
| Slight stain            | 4      |
| Easily noticeable stain | 3      |
| Considerable stain      | 2      |
| Very heavily stained    | 1      |

(The spread or lack of spread is not necessarily reflected in the ratings.)

(d) Duplicate sets of stains were applied in separate areas so that one-half of the fabric could be washed. In most instances, the wash was carried out with 50 grams of "FAB," a cotton cycle, and a dummy load to total 5 pounds in a Norge home automatic washer.

(e) The following two lists describe the numbering and the gross characterizations of the stains employed.

#### Water stains

- (1) Instant tea <sup>1</sup>
- (2) Sheaffer's 232 blue-black Skrip
- (3) A & P Concord grapejuice
- (4) "Ann Page" salad mustard
- (5) "Bosco" chocolate syrup

#### Oil stains

- (6) Wesson Oil
- (7) Gulf "Supreme" motor oil 20/20
- (8) Oleomargarine <sup>2</sup>
- (9) La Rosa tomato sauce
- (10) "Jergen's" lotion

<sup>1</sup> 8 cc. dry powder/200 cc. water applied at 160° F.

<sup>2</sup> Melted and applied at 160° F.

In reporting the relative resistance to staining and ease of stain removal in laundering, the staining values for water-borne and oil-borne stains were averaged separately.

In all cases the stains were allowed to dry on the fabrics for twenty-four hours before laundering.

#### Oily particulate soil repellency (GRC Dry Soil Test)

Fifteen to twenty 6" x 8" numbered specimens (normally 80 x 80 cotton), including at least one untreated control, are tumbled for thirty minutes with 10 percent of "Cyanamid Soil" based on the weight of the fabric. The tumbling is carried out in a 5-liter capacity "Five Minute Home Cleaner" at 44 r.p.m.; six No. 8 neoprene rubber stoppers are distributed among the specimens to increase the mechanical action. At the end of tumbling, the specimens are removed and each shaken separately up and down fifteen times by hand to remove surface dirt.

The specimens are then cut in two (to produce two 4" x 6" pieces). One-half is washed with 50 grams of "FAB" in a cotton cycle with a 5-pound dummy load, then hung to dry and lightly ironed under a clean cotton cloth.

The degree of soiling is determined with a photovolt reflectance meter (tri-blue filter). Six readings per specimen are made and the arithmetic average reported.

The "Cyanamid Soil" described below is the same as that recommended by Minnesota Mining and Manufacturing Co. The following dry ingredients are blended thoroughly, dried in a forced draft convection oven for eight hours at 50° C., then milled for twenty-five hours with ceramic balls and stored in a polyethylene bag.

#### "Cyanamid soil"

| Material:                     | Percent by weight |
|-------------------------------|-------------------|
| Peat moss                     | 38                |
| Cement                        | 17                |
| Kaolin clay <sup>a</sup>      | 17                |
| Silica, 200 mesh <sup>b</sup> | 17                |
| Furnace black <sup>c</sup>    | 1.75              |
| Red iron oxide <sup>d</sup>   | 0.50              |
| Mineral oil                   | 8.75              |

<sup>a</sup> "Peerless," R. T. Vanderbilt.

<sup>b</sup> Davidson Chemical Co.

<sup>c</sup> "Molaco," Benny & Smith Co.

<sup>d</sup> C. K. Williams Co.

It has now been discovered that quaternary ammonium derivatives of highly fluorinated aliphatic carboxylic acids, i.e., aliphatic carboxylic acids in which at least 70 percent to 100 percent of the hydrogen atoms other than the hydrogen of the carboxyl group is replaced with fluorine and in which the terminal or omega carbon atom is attached to two and preferably three fluorine atoms, have the capability of imparting to or conferring upon textiles or textile substrates the resistance to wetting by water or oil, resistance to staining by water-borne or oil-borne stains, and resistance to staining by oily particulate soil. In fact the aforesaid quaternary ammonium derivatives of highly fluorinated aliphatic carboxylic acids shed rather than attract oily particulate soil.

The present quaternary ammonium derivatives of highly fluorinated aliphatic carboxylic acids have compositions corresponding to the generic formula:



where Q is the alkyl moiety of an aliphatic carboxylic acid having three to twenty-one carbon atoms and seven to forty-three hydrogen atoms of which hydrogen atoms at least 70 percent up to 100 percent has been replaced with fluorine atoms and two and preferably three fluorine atoms are attached to the terminal or omega carbon atom of the fluoroalkyl moiety of the fluorinated aliphatic carboxylic acid, m is an integer having a value in the range of one to six and R', R'', and R''' are the same or different lower alkyl groups having one to six carbon atoms. The aforesaid quaternary ammonium derivatives of aliphatic carboxylic acids having four to twenty-two carbon atoms in the molecule including the carboxyl carbon usually are obtained as the salt of an anion such as halide, sulfate, etc., corresponding to the formula:



where Q, R', R'', R''' and m have the same significance as in (B) supra, and An is an anion such as chlorine, bromine, iodine, ethosulfate, etc. The quaternary ammonium derivatives of the present invention are characterized by having an amido as well as an amino-nitrogen.

In general, the quaternary ammonium derivatives of the aliphatic carboxylic acids are prepared by the reactions of classical organic chemistry. For example, the lower alkyl ester of highly fluorinated aliphatic carboxylic acid is reacted with dialkyl aminoalkyl amine in equimolar proportions, the alcohol produced in the reaction removed preferably at less than atmospheric pressure to obtain the intermediate amino-amide as a bottoms product, and the amino-amide reacted with an alkyl halide, preferably the bromide, to obtain the quaternary ammonium derivative of the highly fluorinated aliphatic carboxylic acid.

The mechanism of this particular method, of the several classical methods, of preparing these quaternary

ammonium compounds is represented by the following equations:



Illustrative of the preparation of the quaternary ammonium derivatives of highly fluorinated aliphatic carboxylic acids is the preparation of highly fluorinated, i.e., pentadecafluoroctyl amidopropyl dimethylethyl ammonium bromide. Thus, about 0.15 mol of the butyl ester of pentadecafluoroctanoic acid and about 0.15 mol of dimethyl aminopropylamine were reacted at a temperature in the range of 23° C. to 40° C. for about seven hours. The butanol evolved was distilled at a reduced pressure to obtain the intermediate amino-amide as a bottoms product in a yield of eighty-two percent of theoretical. Thirty parts by weight of the aforesaid amino-amide intermediate were reacted with 9.2 parts by weight (about 0.085 mol) of ethyl bromide in thirty-five parts by weight of methanol for about four hours at a temperature in the range of 28° to about 80° C. A yield of 100 percent of theoretical of the pentadecafluoroctylamido propyldimethylethylammonium bromide was obtained. The bromide of the quaternary ammonium derivative of pentadecafluoroctanoic acid was soluble in water and ethanol.

The foregoing preparation of pentadecafluoroctylamidopropyl dimethylethyl ammonium bromide is illustrated by the following equations:



where Q is  $CF_3(CF_2)_6$ ,



is



or  $C_{15}F_{15}N_2H_{18}OBr$  (mol wt. 607).

Bromine: Calculated (?). Found (?).

The treatment of textile materials to obtain oil repellency and resistance to soiling by oily particulate soil may be typically carried out by padding the textile to at least 80% wet pickup with the quaternary ammonium com-

pounds of this invention and then curing the so treated textile at a temperature of from room temperature to 350° F. and for a period of time inversely proportioned to the temperature; the time and temperature selected to be equivalent to about 5 minutes at 300° F.

The oil repellency and resistance to soiling by oily particulate soil of the QAC compound or pentadecafluoroctylamidoisopropylidemethylethyl ammonium compound is indicated by the following data.

10

TABLE I

| Percent Solids<br>QACBr | pH  | Cured five minutes at 300° F. |              |    |
|-------------------------|-----|-------------------------------|--------------|----|
|                         |     | Oil                           | Reflectance* |    |
|                         |     |                               | B            | A  |
| 2.0                     | 5.5 | 90                            | 53           | 78 |
| 1.0                     | 5.6 | 100+                          | 52           | 78 |
| 0.5                     | 5.3 | 50                            | 48           | 77 |
| Untreated               |     | 0                             | 32           | 79 |

\*The higher the numerical value the less the adherence of the oily particulate soil.

When the textile is pretreated with 3 percent of a cationic urea-formaldehyde resin such as Uformite 467 available from Rohm and Haas Company and then treated with the aforescribed QAC the resistance to wetting by oil and the shedding of oily particulate soil is as indicated by the following data:

30

TABLE II

| Percent Solids<br>QACB, in water | Cured at Room Temp. |             |    | Cured at 300° F. for<br>five minutes |             |    |
|----------------------------------|---------------------|-------------|----|--------------------------------------|-------------|----|
|                                  | Oil                 | Reflectance |    | Oil                                  | Reflectance |    |
|                                  |                     | B           | A  |                                      | B           | A  |
| 1                                | 0+                  | 47          | 79 | 100+                                 | 55          | 80 |
| Untreated                        | 0                   | 31          | 79 | 0                                    | 31          | 79 |

It will be observed that in both treatments the treated cloth (80 x 80 cotton) shed the oily particulate soil before washing as indicated by the values of 31 and 32 for the untreated cloth before washing and the values of 48, 47, and 55 for the treated cloth before washing.

The quaternary ammonium compounds of the present invention, i.e., the highly fluorinated quaternary ammonium derivatives of the highly fluorinated aliphatic carboxylic acids are recovered as the salts thereof having compositions corresponding to the formula:



wherein Q is the alkyl moiety of an aliphatic carboxylic acid having three to twenty-one carbon atoms and seven to forty-three hydrogen atoms of which hydrogen atoms seventy to one hundred percent has been replaced with fluorine atoms and two and preferably three fluorine atoms are attached to the terminal or omega carbon atom; m is an integer in the range of one to six inclusive; R', R'', and R''' are the same or different lower alkyl groups having one to six carbon atoms; and where in Formula C An is an anion e.g., chlorine, bromine, iodine, ethosulfate, and the like, are not to be confused with quaternary ammonium compounds described in the prior art. Thus, for example, in U.S. Patent No. 2,727,923 quaternary ammonium compounds conforming to the formula:



where n is an integer in the range of three to nine; R, R',

and  $R''$  are the same or different alkyl groups having one to five carbon atoms; and  $x$  is a halogen or hydroxyl clearly are not aminoalkylamido derivatives of highly fluorinated aliphatic carboxylic acids.

Similarly, U.S. Patent No. 2,146,392 contains the description of quaternary ammonium salts having compositions corresponding to the formula:



where  $R$  is an aliphatic hydrocarbon radical having two to seventeen carbon atoms;  $N$  (tertiary) is the nucleus of a molecule of pyridine, a *c*-alkylpyridine or quinoline; and  $X$  is a monovalent anion.

It is manifest that the quaternary ammonium compounds described in U.S. No. 2,146,392 are not aminoalkylamido derivatives of highly fluorinated aliphatic carboxylic acids.

Quaternary ammonium salts of cellulose have also been described in the prior art. Thus, in U.S. Patent No. 2,768,162 there is the disclosure of a quaternary ammonium salt of an aminoalkylether of cellulose represented by the formula:



where  $R'$  and  $R''$  are hydrogen or aminoalkyl;  $R''''$ ,  $R'''$ ,  $R'''''$  are alkyl or aralkyl;  $n$  is an integer of from two to four; and  $X$  is any anion.

Quite clearly the quaternary ammonium fraction of the aminoalkylether described in this patent is not aminoalkylamide derivative of an aliphatic carboxylic acid nor of a highly fluorinated aliphatic carboxylic acid.

In U.S. Patent No. 2,878,144 a fabric coated with quaternary ammonium salts of fatty acid esters of a polyhydroxypolyamine is described. This coating material is not an aminoalkylamido derivative of a highly fluorinated aliphatic carboxylic acid.

Thus, the quaternary ammonium salts of the present invention are not described in the prior art.

What is claimed is:

1. Aminoalkylamido derivatives of highly fluorinated aliphatic carboxylic acids having compositions corresponding to the formula:



where  $Q$  is a hydrocarbon radical having three to twenty-one carbon atoms and seven to forty-three hydrogen atoms of which hydrogen atoms at least 70 percent to 100 percent has been replaced with fluorine atoms and at least two fluorine atoms are attached to the terminal carbon atom;  $R'$  and  $R''$  are alkyl groups having one to six carbon atoms;  $m$  is an integer from 1 to 6.

2. Quaternary ammonium derivatives of compounds as defined in claim 1 corresponding to the formula:



where  $R'''$  is an alkyl group having 1 to 6 carbon atoms and  $An$  is an anion,

3. Pentadecafluorooctylamidopropyldimethylamine,



4. Pentadecafluorooctylamidopropyldimethylethylamine hydroxide, having the formula



5. A bromide salt of the quaternary ammonium hydroxide of claim 4.

6. Textile having affixed thereto at least one quaternary ammonium salt as defined in claim 2.

7. Cotton haxing affixed thereto at least one quaternary ammonium salt as defined in claim 2.

8. Textile associated with cationic resin and having a surface comprising at least one quaternary ammonium derivative as defined in claim 2.

9. A method of imparting capability to shed oily particulate soil to textile material which comprises padding textile material to at least 80 percent wet pick-up with

30 at least one amidoalkyltrialkyl ammonium derivative of highly fluorinated aliphatic carboxylic acid having four to twenty-two carbon atoms in which at least 70 percent to 100 percent of the alkyl hydrogens of said aliphatic carboxylic acid has been replaced by fluorine atoms and 35 at least two fluorine atoms are attached to the terminal carbon atom, and curing the so-treated textile at a temperature in the range of room to 350° F. for a period of time inversely proportioned to the temperature and about five minutes at 300° F.

40 10. A method of imparting capability to shed oily particulate soil to textile material which comprises padding textile material with at least one cationic resin, padding the so-treated textile to at least 80 percent wet pick-up with at least one amidoalkyltrialkyl ammonium derivative

45 of highly fluorinated aliphatic carboxylic acid having four to twenty-two carbon atoms in which at least 70 percent to 100 percent of the alkyl hydrogens has been replaced by fluorine atoms and at least two fluorine atoms are attached to the terminal carbon atom, and curing 50 the so-treated textile at a temperature in the range of room to 350° F. for a period of time inversely proportioned to the temperature and about five minutes at 300° F.

#### References Cited

#### UNITED STATES PATENTS

|           |         |                |             |           |
|-----------|---------|----------------|-------------|-----------|
| 2,727,423 | 12/1955 | Husted         | -----       | 260—567.6 |
| 2,743,297 | 4/1956  | Husted et al.  | -----       | 260—561   |
| 2,878,144 | 3/1959  | Conbere et al. | 117—139.5 X |           |
| 2,878,273 | 3/1959  | Conbere et al. | 117—139.5 X |           |
| 3,019,261 | 1/1962  | Pascal         | -----       | 260—56.1  |
| 3,232,790 | 2/1966  | Enders et al.  | 117—139.5   |           |

WILLIAM D. MARTIN, Primary Examiner.

65 T. G. DAVIS, Assistant Examiner.